

Feb. 9, 1926.

1,572,475

F. C. FRARY

REFRACTORY LINING FOR CRUCIBLES AND THE LIKE

Filed Jan. 15, 1924

*Fig. 1.*



*Fig. 2.*



INVENTOR

Francis C. Frary

BY

Cooper, Kerr & Dunham

ATTORNEY

Patented Feb. 9, 1926.

1,572,475

# UNITED STATES PATENT OFFICE.

FRANCIS C. FRARY, OF OAKMONT, PENNSYLVANIA, ASSIGNOR TO ALUMINUM COMPANY OF AMERICA, OF PITTSBURGH, PENNSYLVANIA, A CORPORATION OF PENNSYLVANIA.

## REFRACTORY LINING FOR CRUCIBLES AND THE LIKE.

Application filed January 15, 1924. Serial No. 686,278.

To all whom it may concern:

Be it known that I, FRANCIS C. FRARY, a citizen of the United States of America, residing at Oakmont, in the county of Allegheny and State of Pennsylvania, have invented certain new and useful Improvements in Refractory Linings for Crucibles and the like, of which the following is a full, clear, and exact description.

10 In producing copper-aluminum-silicon alloy by electrothermal reduction of alumina and silica the furnace temperatures range as high as 2000° C. or higher, and in consequence the alloy is so hot when tapped from the furnace into the crucible, ladle, or other receptacle provided to receive it, that receptacles of ordinary construction or material have been found practically useless for the purpose. A furnace operating on power around 1500 kw. will produce as high as two tons of alloy per tapping, and hence the crucible must be mechanically strong enough to sustain and transport such a load. Further, the surface in contact with the molten alloy must not be melted or attacked by the alloy at the high temperatures encountered, since such melting or attack would not only destroy the crucible or the lining thereof but might also contaminate the alloy itself 30 and thereby impair its quality. A steel shell lined with carbon answers the purpose for only a few tappings, since the violent temperature changes produced by the rapid inflow of such quantities of intensely hot metal cause the lining to crack, even though it be preheated. This cracking may be due in part to compressive strains produced in the lining by the stresses incident to lifting and transporting the loaded crucible. But 40 in any case the cost of frequent relining is prohibitive. Fire brick and other refractories such as used for lining crucibles employed in the iron and steel industry are fused by and react with the aluminum-copper-silicon alloy at the temperatures referred to, so that the lining itself is rapidly destroyed and the alloy seriously contaminated.

Of the various materials tried I have 50 found that a lining made of a mixture of alumina and a dilute solution of sodium silicate answers the requirements in a highly satisfactory manner. Such a mixture is cheap, and durable enough to stand

long use. It is also refractory, non-combustible, and is substantially inert to the alloy even at the high temperature at which the latter is tapped. Any form of alumina may be used, but I prefer alumina which has been produced by electrothermal reduction of iron, silicon, titanium and other oxids present as impurities in the original bauxite or other material, leaving the major portion of the alumina unreduced. A method of producing alumina in this manner is described in the copending application of William Hoopes, Junius D. Edwards and myself, Serial No. 608,283, filed December 21, 1922. This product appears to be denser than the alumina obtained by calcination of aluminum hydrate precipitated from sodium aluminate solutions, and when finely divided its sharper and more angular particles pack together better and are more securely bound by the sodium silicate.

Referring to the accompanying drawing, Fig. 1 is a side view, partly in section, illustrating a crucible lined with alumina and sodium silicate mixture.

Fig. 2 is a cross section, on line 2—2 of Fig. 1, illustrating the process of lining the crucible shell according to the preferred method.

The crucible shown comprises a steel shell 10, which may be about 36 to 42 inches in diameter and about 30 inches high. The lining, 11, may be 4 to 6 inches thick. Around the outside of the shell is a steel band 12, having trunnions 13 for lifting and tilting purposes.

In the preferred method of carrying out my invention the alumina is ground to the fineness of ordinary sand and is mixed with dilute sodium silicate solution, say of about 20° Baumé, in amount sufficient to give the mixture a consistency about like that of ordinary molding sand. The steel shell having been prepared I tamp firmly on the bottom a layer 14, Fig. 2, of the alumina and sodium silicate mixture, of suitable thickness. Then placing in the shell a steel form 14 of the proper size and shape, preferably with a slight downward taper to facilitate removal, the annular space between the form and the shell is filled with the lining mixture, which is rammed tightly in place. The form is now removed, lifting

it out by means of the ears 15, after which the crucible is set aside to dry slowly. It is baked at a low temperature, say about 200° C., to drive off the last of the water. The lining thus produced, composed of fine particles of aluminum oxide bound together by sodium silicate, is hard and strong, enabling it to withstand the mechanical stresses incident to even rough usage in the rapid handling and transportation of large quantities of molten metal. It is very refractory, being infusible at temperatures encountered in the use described, and can stand sudden and extreme temperature changes without cracking. At the same time neither it nor the highly heated alloy is injured by contact with each other, even though the alloy contains a metal (in the present instance aluminum) which has a very high affinity for oxygen.

I have also found the mixture highly

advantageous in other places where a refractory lining is desired which will stand high temperatures and sudden temperature changes without cracking, especially where 25 resistance to chemical or other attack by superheated aluminum-copper-silicon alloy is a requisite; as for example the tapping spout or trough of a furnace in which such alloy is produced or melted. For such purposes the mixture described is markedly superior to the customary magnesite composition.

I claim:

A hollow article for handling highly 35 heated aluminum alloy, comprising a steel shell and a lining therein composed essentially of fine particles of solidified alumina bound together by sodium silicate.

In testimony whereof I hereto affix my 40 signature.

FRANCIS C. FRARY.